

1

3,067,028

## Mg-Si-Zn EXTRUSION ALLOY

George S. Foerster, Midland, Mich., assignor to The Dow Chemical Company, Midland, Mich., a corporation of Delaware  
No Drawing. Filed Apr. 27, 1960, Ser. No. 24,889  
3 Claims. (Cl. 75—168)

The invention relates to a magnesium-base alloy and more particularly relates to an improved magnesium-base extrusion alloy containing silicon and zinc. These alloys can be extruded at speeds as high as 100 feet per minute.

Heretofore, the magnesium-aluminum-zinc alloys have been employed as the principal extrusion alloys because they are readily extruded at speeds up to 75 feet per minute, they exhibit moderately high physical properties in the extruded form and they are prepared using low cost alloying elements.

However, the conventional alloy AZ31B containing nominally 3 percent of aluminum, 1 percent of zinc, at least 0.2 percent of manganese and the balance magnesium, is not weldable without stress relief. Upon lowering the aluminum content of a magnesium-aluminum-zinc alloy the physical strength properties of the extruded alloy are found to be inferior to those of AZ31B. Such is the case with the magnesium-base alloy AZ11 which contains nominally 1 percent of aluminum, 1 percent of zinc, the balance magnesium.

In considering other possible magnesium-base extrusion alloys it is well recognized that the addition of increasingly larger proportions of zinc to magnesium, or a magnesium-base alloy, tends to increase the strengths of the resulting alloy. Typical trends are illustrated by the strength properties listed in Table I for extrudes formed of magnesium-zinc binary alloys. The data in the table show the expected increase in properties with increasingly larger proportions of zinc in the alloy and lower properties at higher extrusion speeds.

Other alloys such as the magnesium-aluminum-zinc alloys are known to behave similarly.

2

It has now been discovered that the strength properties of a magnesium-base alloy containing silicon and zinc are unexpectedly enhanced by providing a reduced amount of zinc, i.e. below about 1.5 percent by weight, in combination with a silicon content in the range of 0.2 to 2 percent by weight.

The alloy of the invention is readily prepared according to methods well understood in the magnesium metal art. Magnesium is melted under a conventional flux cover and the requisite amount of silicon and zinc added to the melt while the melt is at a temperature of about 1600° F.

Ferrosilicon is usually the source of silicon, although other forms of silicon such as silicon metal may be used, if desired. In the event ferrosilicon is employed, iron, which is sparingly soluble in molten magnesium, normally precipitates into the bottom sludge layer of the melt. While the zinc may be added to the melt at any time, if ferrosilicon is the source of silicon, the requisite amount of the zinc is added to the melt as metallic zinc after the iron settles out.

After the addition of the alloying components, the melt is brought to casting temperatures, usually in the range of 1250 to 1450° F., and cast into billets suitable for extrusion stock.

The role of the alloying elements is not entirely understood, but it is believed that the silicon addition precipitates in the casting as the finely divided intermetallic compound, magnesium silicide. Magnesium silicide has a very low solid solubility in magnesium and helps to maintain the alloy in the fine-grained condition as well as to increase the strength of the alloy. The silicon content of the alloy of the invention should be as high as feasible, preferably from 0.5 to 1.5 percent.

The presence of zinc greatly improves the corrosion resistance of the alloy and therefore at least 0.2 percent of zinc should be employed. On the other hand at higher zinc levels, such as above about 1.5 percent of zinc, the tensile yield strength, compression yield strength, and ultimate tensile strength of the alloy are decreased. To impart ductility and to improve the surface of the ex-

TABLE I

| Composition, weight percent |       | Extrusion speed, ft./min. | Form of extrude | Cross-sectional dimensions, inches | Percent E | Strengths in 1,000 p.s.i. |     |    |
|-----------------------------|-------|---------------------------|-----------------|------------------------------------|-----------|---------------------------|-----|----|
| Zn                          | Zr    |                           |                 |                                    |           | TYS                       | CYS | TS |
| 0.9                         | ----- | 3                         | Rod             | 3/8 diameter                       | 16        | 21                        | 12  | 35 |
| 1.9                         | ----- | 3                         | Rod             | 3/8 diameter                       | 18        | 23                        | 13  | 35 |
| 1.3                         | 0.6   | 12                        | Rod             | 3/8 diameter                       | 18        | 38                        | 29  | 45 |
| 2.4                         | 0.6   | 12                        | Rod             | 3/8 diameter                       | 18        | 40                        | 33  | 50 |
| 1.3                         | 0.6   | 12                        | Strip           | 1/16 x 3/4                         | 5         | 38                        | 29  | 44 |
| 2.4                         | 0.6   | 12                        | Strip           | 1/16 x 3/4                         | 6         | 40                        | 38  | 47 |
| 1.3                         | 0.6   | 20                        | Strip           | 1/16 x 3/4                         | 6         | 34                        | 19  | 40 |
| 2.4                         | 0.6   | 20                        | Strip           | 1/16 x 3/4                         | 8         | 38                        | 29  | 26 |
| 1.3                         | 0.6   | 40                        | Strip           | 1/16 x 3/4                         | 11        | 27                        | 15  | 37 |
| 2.4                         | 0.6   | 40                        | Strip           | 1/16 x 3/4                         | 12        | 31                        | 20  | 43 |

<sup>1</sup> Balance magnesium.

NOTE.—Percent E=Percent elongation in 2 inches. TYS=Tensile yield strength. CYS=Compression yield strength. TS=Ultimate tensile strength.

In the German Patent 519,377 there is described a magnesium-base alloy containing from 1.8 to 5 percent by weight of zinc and from 1 to 6 percent by weight of silicon. The alloy of the German patent is said to be useful when cast as pistons for internal combustion engines. An example of this alloy such as one containing 4 percent by weight of zinc and 1.5 percent by weight of silicon, the balance magnesium is not, however, suitable as an extrusion alloy because it tends to crack on being welded, it cannot be extruded at speeds above about 30 feet per minute, and an extrude of the alloy does not exhibit the level of strength properties desirable in an extruded product.

trude without adversely affecting weldability the zinc content of the alloy should preferably be in the range of 0.5 to 1.3 percent and more desirably about 1 percent.

It has also been found that various additional alloying elements may be added to the magnesium-silicon-zinc alloy of the invention to advantageously modify the properties of this alloy for special purposes.

An especially desirable additional alloying element is manganese. The addition of small amounts of manganese permits the use of a lower silicon content without loss of mechanical strength. This is often advantageous as silicon tends to not alloy efficiently with molten magnesium, and lower silicon contents are more easily ob-

tained. Up to 1.5 percent by weight of manganese can be incorporated into the alloy to increase the mechanical strength and corrosion resistance thereof. A preferred composition is one containing by weight, about 1 percent of silicon, about 1 percent of zinc, about 0.4 percent of manganese, the balance magnesium.

Beryllium in an amount up to 0.05 percent by weight may be added to increase matrix strength and to improve resistance to oxidative attack by the atmosphere. Up to 0.5 percent of misch metal may be added to increase matrix strength and cold workability. Up to 0.5 percent of calcium may be added to increase matrix strength where some brittleness may be tolerated. Up to 0.1 percent of zirconium may be added to obtain beneficial grain refining action. And, up to 3 percent of aluminum may be added to improve the surface appearance of the resultant extrude.

Magnesium-silicon-zinc alloys prepared in accordance with the invention can be extruded at speeds as high as 100 feet per minute and at reduction ratios as great as 150 to 1. Extrusion speed does not ordinarily adversely affect the physical properties of the extruded material nor is the extrusion subject to hot shorts.

#### EXAMPLES

In accordance with the present invention, a series of magnesium-silicon-zinc alloys were prepared by alloying together the requisite proportions of magnesium, ferrosilicon, and zinc metal. The resulting alloys were separated from the precipitated iron and each cast as 3 inch diameter billets. The cooled solidified billets were scalped, heated to about 700° F., placed in a preheated ram-extrusion press, and extruded at a temperature of about 600° F. and at speeds in the range of 5 to 100 feet per minute. The physical properties of the resulting extrusions were measured. In Table II are listed the physical properties for 2 alloys of the invention which were each extruded at different speeds. The data show that high extrusion speed is not deleterious but even beneficial to the physical properties of the extruded product.

TABLE II

## Effect of Extrusion Speed

| Run No. | Composition, <sup>1</sup> percent |     | Extrusion speed, feet/minute | Physical properties of extrude |              |     |    |  |
|---------|-----------------------------------|-----|------------------------------|--------------------------------|--------------|-----|----|--|
|         | Si                                | Zn  |                              | Percent E                      | 1,000 p.s.i. |     |    |  |
|         |                                   |     |                              |                                | TYS          | CYS | TS |  |
| 1       | 0.5                               | 1   | 5                            | 15                             | 21           | 15  | 35 |  |
| 2       | 0.5                               | 1   | 20                           | 14                             | 22           | 16  | 36 |  |
| 3       | 0.5                               | 1   | 50                           | 14                             | 23           | 16  | 37 |  |
| 4       | 0.5                               | 1   | 100                          | 14                             | 23           | 16  | 37 |  |
| 5       | 1.2                               | 0.5 | 5                            | 8                              | 24           | 17  | 37 |  |
| 6       | 1.2                               | 0.5 | 20                           | 9                              | 25           | 17  | 38 |  |
| 7       | 1.2                               | 0.5 | 50                           | 9                              | 26           | 19  | 33 |  |
| 8       | 1.2                               | 0.5 | 100                          | 10                             | 27           | 18  | 38 |  |

<sup>1</sup> Composition in weight percent, balance magnesium.

The physical properties of other alloys of the invention which were extruded at 100 feet per minute are listed in Table III. Some of the alloys listed in Table III were also tested to determine their resistance to corrosion. In these instances corrosion tests of one week duration were carried out by the alternate immersion method according to which test specimens are repeatedly immersed for 30 seconds in a 3 percent aqueous sodium chloride solution maintained at 95° F., then withdrawn from the chloride solution for 90 seconds on a two minute cycle according to ASTM standard I-B (B 192-44T).

By way of comparison extrudes formed, respectively, of a magnesium-silicon binary alloy, of a magnesium-zinc binary alloy, and of the conventional alloys AZ31B and AZ11 were tested to determine their physical properties and corrosion resistance. The results of these additional tests are also listed in Table III for comparison.

In accordance with the invention, a further series of magnesium-silicon-zinc alloys containing a fourth alloying element selected from the group consisting of manganese, misch metal, calcium, zirconium, beryllium, and

TABLE III

| Run No.    | Composition, <sup>1</sup> percent |     |     |    | Extrusion speed, feet/min. | Physical properties                     |              |     |                      |  |
|------------|-----------------------------------|-----|-----|----|----------------------------|-----------------------------------------|--------------|-----|----------------------|--|
|            | Si                                | Zn  | Al  | Mn |                            | Percent E                               | 1,000 p.s.i. |     |                      |  |
|            |                                   |     |     |    |                            |                                         | TYS          | CYS | TS                   |  |
| 9          | 1.4                               | 1.0 |     |    | 100                        | 10                                      | 25           | 17  | 37                   |  |
| 10         | 1.0                               | 1.0 |     |    | 100                        | 12                                      | 24           | 17  | 37                   |  |
| 11         | 0.5                               | 1.0 |     |    | 100                        | 14                                      | 23           | 16  | 36                   |  |
| 12         | 1.5                               | 0.5 |     |    | 100                        | 9                                       | 26           | 18  | 38                   |  |
| 8          | 1.2                               | 0.5 |     |    | 100                        | 10                                      | 27           | 18  | 38                   |  |
| 13         | 1.4                               | 1.0 |     |    | 100                        | 10                                      | 26           | 18  | 38                   |  |
| 14         | 1.2                               | 1.0 |     |    | 100                        | 12                                      | 25           | 17  | 37                   |  |
| 15         | 0.9                               | 1.0 |     |    | 100                        | 13                                      | 24           | 17  | 37                   |  |
| 4          | 0.5                               | 1.0 |     |    | 100                        | 14                                      | 23           | 16  | 37                   |  |
| 16         | 1.3                               | 1.5 |     |    | 100                        | 10                                      | 23           | 17  | 36                   |  |
| Comparison | 1.4                               |     |     |    | 100                        | 5                                       | 22           | 17  | 37                   |  |
| Do         | 1                                 | 3   | 0.4 |    | 50                         | 15                                      | 29           | 14  | Ca. 20               |  |
| Do         | 0.6                               | 1.3 | 0.3 |    | 100                        | 11                                      | 23           | 11  | Ca. 0.4              |  |
| Do         | 1                                 |     |     |    | 60                         | 8                                       | 14           | 7   | ( <sup>2</sup> ) 1-6 |  |
| Do         | 1.4                               | 2.0 |     |    | 100                        | 9                                       | 22           | 16  | Ca. 1                |  |
| Do         | 1.4                               | 3.9 |     |    | 25                         | 10                                      | 21           | 15  | 35                   |  |
| Do         | 1.4                               | 3.9 |     |    | 50                         | Very poor, severely cracked as extruded |              |     |                      |  |

<sup>1</sup> Composition in weight percent, balance magnesium.

<sup>2</sup> Typical range.  
NOTE.—Percent E=Percent elongation in 2 inches. TYS=Tensile yield strength in thousands of p.s.i. CYS=Compression yield strength in thousands of p.s.i. TS=Ultimate tensile strength in thousands of p.s.i. M/C/D=Milligrams corrosion loss per sq. centimeter of surface area per day.

aluminum, were prepared by alloying together the requisite proportions of magnesium, ferrosilicon, zinc and the fourth metal. The resulting alloys were separated from the precipitated iron and each cast as 3 inch diameter billets. The cooled solidified billets were scalped, and heated to about 700° F. and placed in a pre-heated ram extrusion press and extruded at a temperature of about 600° F. and at speeds in the range of 5 to 100 feet per minute. The physical properties of the resulting extrusions were determined and are listed in Table IV.

TABLE IV

| Run No. | Composition, <sup>1</sup> percent |     |       |       |         |       |       | Extrusion speed, feet/min. | Physical properties |              |    |    |
|---------|-----------------------------------|-----|-------|-------|---------|-------|-------|----------------------------|---------------------|--------------|----|----|
|         | Si                                | Zn  | Be    | Mn    | Zr      | Al    | MM    |                            | Percent E           | 1,000 p.s.i. |    |    |
|         |                                   |     |       |       |         |       |       |                            | TYS                 | CYS          | TS |    |
| 17...   | 1.5                               | 1.0 | 0.01  | ----- | -----   | ----- | ----- | 100                        | 10                  | 26           | 18 | 37 |
| 18...   | 1.2                               | 0.2 | ----- | 0.3   | -----   | ----- | ----- | 100                        | 8                   | 30           | 18 | 39 |
| 19...   | 1.0                               | 0.3 | ----- | 0.3   | -----   | ----- | ----- | 100                        | 7                   | 30           | 19 | 41 |
| 20...   | 0.4                               | 1.0 | ----- | 0.4   | -----   | ----- | ----- | 100                        | 12                  | 22           | 14 | 36 |
| 21...   | 0.9                               | 1.0 | ----- | 0.4   | -----   | ----- | ----- | 100                        | 12                  | 26           | 13 | 39 |
| 22...   | 1.4                               | 1.0 | ----- | 0.2   | -----   | ----- | ----- | 100                        | 8                   | 25           | 13 | 37 |
| 23...   | 1.5                               | 1.0 | ----- | ----- | -----   | 0.05  | ----- | 100                        | 9                   | 24           | 17 | 36 |
| 24...   | 1.4                               | 1.0 | ----- | ----- | Tr.<.01 | ----- | ----- | 100                        | 8                   | 24           | 18 | 37 |
| 25...   | 1.7                               | 0.9 | ----- | ----- | -----   | 0.9   | ----- | 100                        | 6                   | 21           | 15 | 32 |
| 26...   | 1.4                               | 1.0 | ----- | ----- | -----   | 3.0   | ----- | 100                        | 8                   | 20           | 14 | 33 |

<sup>1</sup> Composition in weight percent, balance magnesium.

NOTE.—Percent E=Percent elongation in 2 inches. TYS=Tensile yield strength in thousands of p.s.i.

CYS=Compression yield strength in thousands of p.s.i. TS=Ultimate tensile strength in thousands of p.s.i.

MM=Misch metal, a mixture of rare earth metals; the mixture used contained about 50 percent of cerium.

Among the advantages of the alloy of the invention are the improved corrosion resistance and ductility that it exhibits compared to that of magnesium-silicon binary alloys.

This application is a continuation-in-part of a prior filed application, Serial No. 819,814, filed June 12, 1959, now abandoned.

from 1 to 1.5 percent by weight of silicon, about 1 percent by weight of zinc, the balance being essentially magnesium.

#### References Cited in the file of this patent

#### FOREIGN PATENTS

40,937 Denmark ----- Oct. 4, 1929  
40,937 Italy ----- Mar. 3, 1945